

June 6, 1933.

E. P. ARPIN, JR.

1,913,017

## METHOD OF TREATING PAPER

Filed June 29, 1931



EDMUND P. ARPIN, JR.

Charles H. Teller

bus-

~~ATTUS~~

## UNITED STATES PATENT OFFICE

EDMUND P. ARPIN, JR., OF PORT EDWARDS, WISCONSIN, ASSIGNOR TO NEKOOSA-  
EDWARDS PAPER COMPANY, OF PORT EDWARDS, WISCONSIN, A CORPORATION OF  
WISCONSIN

## METHOD OF TREATING PAPER

Application filed June 29, 1931. Serial No. 547,558.

This invention relates to a method for treating web material such as paper to increase the strength of the web.

More specifically this invention relates to the preparation of creped paper.

It is an object of this invention to increase the mullen and tensile strength of a web material by subjecting the web to a process which is economical and which may 10 be carried out with apparatus having a low initial cost.

It is a further object of this invention to provide a simple and efficient process for preparing impregnated creped paper.

15 It is a further object of this invention to prepare a creped sheet material which holds its shape and is not readily decrinkled.

Other and further objects of this invention will be apparent from the following 20 description and appended claims.

This invention (in a preferred form) is illustrated in the accompanying drawing and hereinafter more fully described.

On the drawing:

25 Figure 1 is a side elevational view of the left hand end of the apparatus used in carrying out the process of this invention.

Figure 2 is a side elevational view of the right hand end of the apparatus as shown 30 in Figure 1.

As shown on the drawing:

The reference numeral 1 indicates a web from a roll 2 which is passed over rollers 3 into a tub 4 containing a sizing composition. The web material 1 after passing over the guide rolls 3 is directed under a doctor roll 6 immersed into the sizing solution in the tank 4. The web 1 is then passed between rolls 5 and 6 to spread the sizing material uniformly over the sheet. The web 40 is then directed back again into the sizing bath in the tub 4 by passing it around a roll 7. The rolls 5, 6, and 7 may be supported in any suitable manner such as for example 45 by mounting them in a frame. The support has not been illustrated in the drawing and the rolls are shown diagrammatically for clearness.

The web is passed through a second pair 50 of rolls 9 and 10 wherein the excess sizing

material is removed. It should be understood that the number of press rolls may be varied according to the particular need in carrying out the process. Two sets are shown in the drawing but in some cases one 55 set of press rolls is sufficient whereas in other instances it is found desirable to insert three or even more pairs of rolls.

The sized sheet is in a moist or damp condition from the passage through the sizing 60 bath and has a tendency to adhere to roll 9. A creping attachment consisting of a stub blade 11 and a small auxiliary roll 12 are suitably mounted to press against the roll 9. The roll 12 is mounted a short distance 65 above the blade 11 so as to press against the web immediately preceding its contact with the blade 11. The moistened sheet on the roll 9 prior to its contact against the stub blade 11 adheres to the roll 9 and upon 70 reaching the blade 11 is scraped therefrom thus causing the paper to become crinkled or creped. The tenacity with which the moistened sized sheet adheres to the roll 9 greatly aids the creping action of the scraper 75 blade.

The now creped web 1 is passed onto a wire or endless conveyor belt 13. The wire or conveyor belt 13 is directed around rollers 14 and 15 which are driven by any suitable means such as for example by a belt 80 drive from a main driving roll 16.

A spraying device 17 is positioned after the creping attachment so as to direct a spray upon the creped sheet as it moves 85 along the conveyor belt 13. The spraying device 17 may be of any suitable make but I prefer to use a device similar to that described in my copending application Serial No. 135,729, filed September 16th, 1926. 90

A heater 18 is suitably supported as by a frame 18' positioned a short distance beyond the conveyor belt supporting roll 14. An air duct 19 is suitably connected to the heater 18 and extends therefrom over the traveling web 1. The air duct 19 is provided with a number of baffles 20 spaced at intervals along its lower periphery so as to direct the current of heated air from the heater 18 which is provided with a blowing de- 95 100

vice downwardly against the traveling web 1 so as to dry the web. The air duct 19 is tapered as shown at 21 so that the air directed toward the web will be uniform throughout the total extent of travel of the web. A second conveyor wire or belt 22 directed around pulleys 23 and 24 which are suitably journaled in frames 25 and 26 respectively is provided for conveying the web 1 under a second set of heaters. This second conveyor belt may be driven from the first belt by means of a suitable driving belt or chain 27 positioned around pulleys 14 and 23.

15 A second heating unit comprising a pair of heaters 28 and 29 mounted on supports 25 and 26 is provided for heating the partially dried web from the lower conveyor belt 13. The heater units 28 and 29 may be any one of the numerous types of commercial air heaters on the market and may be heated by any suitable means. A large elongated duct 30 tapered so that its greatest cross sections are at the ends thereof and its smallest cross section is at the middle extends from heater 28 to heater 29. The air duct 30 is provided with a number of baffles 31 and 32 which are placed at spaced intervals along its lower periphery. 30 The baffles extend upwardly a short distance into the interior of the duct 30. Baffles 31 are inclined toward the heater 28 while baffles 32 are inclined toward the heater 29 to effect a uniform distribution of heated air throughout the entire length of the duct 30. The tapered duct 30 having its smallest cross section at the middle further aids in the uniform distribution of heated air throughout the entire length.

40 A winder roll 33 suitably supported as by the frame 34 is positioned a short distance beyond the heater 29 to receive the treated web 1. The winder roll 33 may be hand operated by means of a crank 35 or any 45 suitable driving means may be used for removing the treated web from the conveyor 22.

To recapitulate briefly the operation of the device in which my process may be effected, a web such as a paper sheet 1 is unrolled from a roll 2 and passed through a size tub 4 which is steam jacketed and may be heated wherein the web is thoroughly impregnated with the sizing material. Upon 50 leaving the size tub the paper web is passed between press rolls 9 and 10 to remove the excess size. The web is scraped from the press roll 9 to form a creped sheet which is allowed to drop on a traveling conveyor wire 13. If 55 desired, the creping operation may be dispensed with and the uncreped sheet fed to the conveyor wire 13. The sheet passes under a spray device 17 while on the conveyor wire and is sprayed with a hardening solution to 60 set the still wet size on the sheet. An ad-

ditional spray device or a plurality of devices may be arranged to direct a spray against the other side of the sheet if desired. However, this is ordinarily not necessary since the spray from unit 17 as shown on the drawing is generally sufficient to penetrate and satisfactorily harden the sized sheet. If the sheet has been creped, the spray hardening treatment at the same time sets the crinkles in the creped sheet and produces a sheet which is not readily de-creped and holds its shape even when placed under considerable tension. After passing the spray the sheet is passed beneath a dryer 19 wherein it is partially dried. It is then next elevated to a conveyor wire 22 where it passes beneath an elongated air duct 30 under which the drying process is finished. The thoroughly dried web is then removed from the conveyor wire 22 at 24 and wound into a roll 33.

While any sizing material may be used in the size bath I prefer to use a solution such as described in my copending Serial No. 563,667, filed September 18, 1931 and having essentially the following composition:

|                                        |                        |     |
|----------------------------------------|------------------------|-----|
| Glue or gelatine                       | 40 to 90% (dry weight) | 80  |
| Glycerine, or other polyhydric alcohol | 0 to 30%               | 90  |
| Liquid rubber latex                    | 1 to 40%               | 95  |
| Triethanolamine or similar substance   | 0 to 30%               | 100 |

It will be seen from the above range of proportions used in the preferred sizing solution that the materials may be varied throughout a wide range. However, in most cases, it is essential that the glue or gelatine content should not be allowed to drop below 60% in order to assure a glazed finish on the paper.

While any hardening solution may be used in the spray treatment I prefer to subject the creped sheets to a spray consisting of a mixture of furfural and formaldehyde. The furfural and formaldehyde may be mixed and sprayed directly on the material or the mixture of furfural and formaldehyde may be diluted by the addition of commercial denatured alcohol and/or distilled water. The spray treatment as pointed out sets the sizing material already impregnated into the web and results in a waterproof coating upon the web. The resulting effect is somewhat similar to that obtained by tanning leather. Either furfural or formaldehyde may be used alone in the spray hardening treatment but I prefer to use a composition consisting of a mixture of 75% furfural and 25% formaldehyde. However other aliphatic aldehydes and ketones may be substituted for the formaldehyde and furfural.

The resulting treated paper has a greatly increased mullen and tensile strength over 130

that of ordinary paper. The paper sheet also has a great resistance to tearing action and a high resistance to penetration of water, oil or similar liquids. The paper has 5 a pliability which will not be lost upon ageing.

It has been found furthermore that paper treated by my process has very good peeling properties from materials of an adhesive nature. This quality makes the treated 10 paper highly desirable for use in making paper backed adhesive tape.

Many changes may be made in the details 15 and arrangement of the apparatus and the steps of the process and I do not wish to be limited otherwise than as necessitated by the prior art and scope of the appended claims.

I claim as my invention:

1. The process of treating paper which 20 comprises passing a web of paper through a bath containing a gelatinous material, a polyhydric alcohol and rubber latex and spraying the web as it emerges from the bath with a solution containing an aldehyde 25 to form a hardened surface on the web.

2. The method of treating web material which comprises passing the said web material through a bath containing a gelatinous material and a polyhydric alcohol, 30 subsequently passing the web through press rolls, creping the web by scraping it from the press rolls, and spraying the creped web with a fluid which reacts with the gelatinous material to set the creped web.

3. The process of treating paper which 35 comprises passing a web of paper through a bath containing a gelatinous material, a polyhydric alcohol and rubber latex, creping the web as it emerges from the bath 40 and coating the material impregnated on the web with an aldehyde to form a hardened surface on the web.

4. The process of treating paper which 45 comprises passing a paper web through a bath having the following composition:

|                     |           |
|---------------------|-----------|
| Glue or gelatine    | 40 to 90% |
| Glycerine           | 0 to 30%  |
| Liquid rubber latex | 1 to 40%  |
| Triethanolamine     | 0 to 30%  |

50 creping the impregnated sheet as it emerges from the bath and spraying the creped sheet with a solution containing 25% formaldehyde and 75% furfural.

55 In testimony whereof I have hereunto subscribed my name at Port Edwards, Wood County, Wisconsin.

EDMUND P. ARPIN, JR.